

# UNITED STATES PATENT OFFICE.

JUDSON RICE AND ANDREW STEIGER, OF SAN JOSÉ, AND ISAAC L. THURBER, OF SANTA CRUZ, CALIFORNIA.

## ASPHALTIC TILING AND PAVING MATERIAL.

SPECIFICATION forming part of Letters Patent No. 322,970, dated July 28, 1885.

Application filed October 2, 1884. (No specimens.)

*To all whom it may concern:*

Be it known that we, JUDSON RICE and ANDREW STEIGER, residing at the city of San José, county of Santa Clara, and ISAAC LANE 5 THURBER, residing at the city and county of Santa Cruz, all in the State of California, have invented a new, useful, and Improved Asphaltic Tiling and Paving Material; and we declare the following to be a specification.

10 Tiling is used for floors, vestibules, and walks, and, when the tile are increased in size, for paving sidewalks and streets.

Heretofore tiling has been made with Portland cement as the principal ingredient, but 15 the composition is expensive. Clay has been used to make an article known as "terra cotta." Marble and natural sandstone have also been used for the purpose of paving sidewalks, vestibules, and walks, but all are expensive, and 20 are liable to crack and break under a light pressure.

The object of our invention is to make an article for the purpose for which cement, clay, stone, and marble are now used for paving and 25 tiling of a much cheaper material and more durable than either, and that will resist pressure without breaking.

To carry out our invention we take asphaltum, which is found in large quantities in California, and form it into the material herein 30 described.

We have discovered that asphaltum in its native state obtains a surface that is hard, smooth, durable, and elastic; but previous to 35 our invention of the process for working and using asphaltum it has had little or no commercial value for the purposes stated. We take the native asphaltum after it has been softened by our process for preparing and 40 working asphaltum, (for which application for

Letters Patent has been filed by us in the Patent Office of the United States,) and after it is in a plastic state we subject it to a pressure in a suitable mold of any desired form, thus forming the tiling and paving material. 45

When the asphaltum is in its plastic state coloring-matter may be mixed with it, and clean sand, if necessary, to give it the proper consistency.

The pressure used may be varied according 50 to the quality of the asphaltum, but the pressure removes all the water which may be in it and any other liquid substance, and gives it a smooth and polished surface.

The tiling thus formed is composed only of 55 native asphaltum, sand, and coloring material.

We are aware that English Patent No. 3,275 of 1873 describes the pulverizing of native asphalt and its subjection without heat to pressure in molds to form blocks, tiles, or slabs of 60 compressed asphalt. We do not claim the material thus produced, it not being of our invention; nor do we claim melted uncompressed asphalt, nor unmelted compressed asphalt, nor asphalt mixed with sawdust, nor mixtures in 65 which asphalt is used to hold clinkers and cinders together, nor mixtures in which sand predominates over asphalt; but

What we do claim is—

A tiling or roofing material consisting of 70 compressed melted native asphalt, substantially pure and having a hard, smooth, durable, and elastic surface, substantially as set forth.

JUDSON RICE.

ANDREW STEIGER.

ISAAC L. THURBER.

Attest:

SAMUEL P. HOWES, Jr.,  
D. D. TENNYSON.